# EUROPEAN PATENT SPECIFICATION

(11) **EP 0 099 948 B1**
(45) Date of publication and mention of the grant of the patent: **20.11.1986**
(21) Application number: 82303995.3
(22) Date of filing: 28.07.1982
(51) Int. Cl.: C22B 21/06

(54) **Process for producing high-purity aluminum**
Verfahren zur Herstellung von Aluminium hoher Reinheit
Procédé pour fabriquer de l'aluminium de grande pureté

(43) Date of publication of application: 08.02.1984
(73) Proprietor: SHOWA ALUMINUM CORPORATION, Sakai Osaka (JP)
(72) Inventor: Shingu, Hideo, Sakyo-ku Kyoto (JP); Arai, Kozo Showa Aluminum Corporation, Sakai Osaka (JP); Sakaguchi, Masashi Showa Aluminum Corporation, Sakai Osaka (JP); Nishide, Toshio Showa Aluminum Corporation, Sakai Osaka (JP); Watanabe, Osamu Showa Aluminum Corporation, Sakai Osaka (JP); Tashiro, Yasushi Showa Aluminum Corporation, Sakai Osaka (JP); Otsuka, Ryotatsu Showa Aluminum Corporation, Sakai Osaka (JP); Tsukamoto, Kenji Showa Aluminum Corporation, Sakai Osaka (JP)
(74) Representative: Drever, Ronald Fergus

## Description

The present invention relates to a process for producing aluminum having high purity, and more particularly to a process for treating aluminum containing eutectic impurities, such as Fe, Si, Cu and Mg, and also peritectic impurities, such as Ti, V and Zr, by resorting to segregation solidification to obtain aluminum having lower contents of eutectic impurities and peritectic impurities and a higher purity than the original aluminum.

Throughout the specification and the appended claims, the term "eutectic impurities" refers to the impurities which undergo a eutectic reaction with aluminum, and the term "peritectic impurities" refers to the impurities which undergo a peritectic reaction with aluminum.

When aluminum containing both eutectic impurities and peritectic impurities is melted and then subjected to equilibrium solidification, the impurity concentration Cs of the resulting solid aluminum fraction is theoretically represented by the following equation. where ko is the distribution coefficient, Co is the impurity concentration of the original aluminum, and fs is the ratio of the solid fraction. The above equation shows that when the distribution coefficient ko is smaller than 1, the impurity concentration Cs of the solid fraction is smaller than the impurity concentration Co of the original aluminum and that when the distribution coefficient ko is larger than 1, the impurity concentration Cs of the solid fraction is greater than the impurity concentration Co of the original aluminum. Since eutectic impurities are smaller than 1 in distribution coefficient, the solid fraction prepared from aluminum containing such impurities is lower than the original aluminum in impurity concentration. Accordingly when the original aluminum is melted and thereafter solidified, high-purity aluminum can be obtained advantageously by selectively separating off the resulting pro-eutectic aluminum. Segregation solidification processes based on this principle are already known as disclosed for example, in U.S. Patents No. 3,671,229, No. 3,211,547, etc. However, peritectic impurities are larger than 1 in distribution coefficient, so that aluminum containing such impurities affords a solid fraction which is higher than the original aluminum in impurity concentration. Accordingly when aluminum containing both eutectic impurities and peritectic impurities is treated by the conventional segregation solidification process to obtain pro-eutectic aluminum selectively, the resulting solid fraction is lower in the concentration of eutectic impurities but higher in the concentration of peritectic impurities than the original aluminum.

Aluminum containing both eutectic impurities and peritectic impurities is therefore usually treated by adding boron to a melt of such aluminum in a container to cause the boron to react with Ti, V, Zr and like peritectic impurities and form insoluble metallic borides such as TiB₂, VB₂, ZrB₂, etc., allowing the mixture to stand for a long period of time, for example, for more than 1 hour to settle the metallic borides, placing the molten aluminum into another container as separated from the borides, and selectively drawing off pro-eutectic aluminum only from the container. This process is inefficient since the settlement of the metallic borides requires much time.

Such aluminum has alternatively been treated by rotation of a cooling body within the molten aluminum as described in JP-A-56-127735.

The object of the present invention is to overcome the above drawback and to provide a process for treating aluminum containing both eutectic impurities and peritectic impurities by segregation solidification to remove the impurities of both types from the aluminum to the greatest possible extent and obtain aluminum having a higher purity than the original aluminum.

According to one aspect of the present invention there is provided a process for producing high-purity aluminum comprising the steps of melting the aluminum to be purified and containing both eutectic impurities and peritectic impurities to obtain molten aluminum, and rotating a cooling body when immersed in the molten aluminum while introducing a cooling fluid to the interior of the cooling body to crystallize high-purity aluminum on the surface of the body, characterised by placing the molten aluminum into a holding container and controlling the temperature of the molten aluminum, adding boron to the molten alumimum within the container, and rotating the cooling body at a predetermined speed when immersed in the molten aluminum containing boron and dispersed borides of peritectic impurities resulting from the boron addition.

With this process, the boron reacts with the peritectic impurities to form metallic borides, which are moved away from the cooling body and dispersed throughout the liquid phase by the centrifugal force produced by the rotation of the cooling body. Accordingly an aluminum fraction having lower contents of eutectic impurities and peritectic impurities than the original aluminum can be crystallized on the surface of the cooling body, giving high-purity aluminum. Unlike the conventional process, the present process does not involve the necessity of settling the metallic borides and therefore can be practiced within a shortened period of time.

When aluminum containing Fe, Si, Cu, Mg and like eutectic impurities, and Ti, V, Zr and like peritectic impurities is melted, and boron is added to the resulting melt, the boron reacts with the Ti, V, Zr and like peritectic impurities to form TiB₂, VB₂, ZrB₂ and like insoluble metallic borides. The amount of boron to be used, which is determined in accordance with the Ti, V, Zr and like contents of the aluminum to be purified, is a predetermined amount larger than the amount needed for forming the above metallic borides. The boron may be added in the form of an Al-B master alloy or NaBF4 or like salt. Since boron undergoes a eutectic reaction with aluminum, the excess of boron other than the quantity of boron forming the metallic borides with the peritectic impurities is removed in the same manner as the eutectic impurities as will be described below.

When a cooling body is rotated as immersed in the boron-containing molten aluminum while introducing a cooling fluid to the interior of the body, high-purity aluminum crystallizes on the surface of the cooling body. Stated more specifically, when aluminum containing eutectic impurities is melted and subjected to equilibrium solidification, pro-eutectic aluminum of high purity separates out first. The ratio between the eutectic impurity concentration of the solid phase and the eutectic impurity concentration of the liquid phase at this time is represented by the distribution coefficient ko. During actual solidification, however, the eutectic impurities are relased into the liquid phase to form a layer of concentrated eutectic impurities in the liquid phase in the vicinity of the liquid-solid interface or boundary, so that the impurity concentration of the solid phase is governed by the effective distribution coefficient k_{E} considering the thickness of the concentrated layer (hereinafter referred to as "diffusion layer"). Thus the impurity concentration Cs of the solid phase is represented by Equation (1) wherein k_{E} is used in place of ko, i.e. by the following equation.

It is already known that the effective distribution coefficient k_{E} is represented by the following equation. wherein R is the solidification velocity, 6 is the thickness of the diffusion layer formed in the vicinity of the liquid-solid interface, and D is the diffusion coefficient of the eutectic impurities in the liquid phase. It therefore follows that the effective distribution coefficient k_{E} can be made approximate to the distribution coefficient ko effectively by decreasing the solidification velocity R and the thickness of the diffusion layer, 6, and increasing the diffusion coefficient D. Of these variables, the diffusion coefficient D is considered to be a constant which is dependent on the kind of the eutectic impurity generally when the liquid phase has a constant temperature, so that it is difficult to vary the diffusion coefficient D. It is therefore effective to decrease the solidification velocity R and the thickness of the diffusion layer, 6, for making the effective distribution coefficient k, approximate to the distribution coefficient ko.

When the eutectic impurities are released into the liquid phase at the liquid-solid interface, dendrites are formed at the interface. It is well known that when such dendrites grow, the impurities released into the liquid phase in the vicinity of the liquid-solid interface are trapped, as they are or in the form of eutectic crystals of several microns, in the interstices of the dendrites. This phenomenon is undesirable for the purification of aluminum. The growth of dendrites occurs when the actual temperature of the liquid phase is lower than the temperature of the equilibrium liquidus in the vicinity of the liquid-solid interface. This phenomenon is referred to as constitutional undercooling. The growth of dendrites is promoted when the difference (degree of undercooling) AT between the temperature of the equilibrium liquidus and the actual liquid phase temperature increases. Accordingly the growth of dendrites can be inhibited effectively by decreasing the difference ΔT. To decrease AT, there is the need to increase the temperature gradient of the melt in the vicinity of the liquid-solid interface. Ideally, the temperature gradient should be smaller than the temperature gradient of the equilibrium liquidus to make AT smaller than 0.

The foregoing leads to the following three requirements for purifying aluminum with improved efficiency.
(a) To decrease the solidification velocity to the greatest possible extent.
(b) To decrease to the greatest possible extent the thickness of the diffusion layer in the vicinity of the liquid-solid interface.
(c) To increase to the greatest possible extent the temperature gradient involved in the liquid phase in the vicinity of the interface.

When a cooling body is immersed in molten aluminum containing boron, aluminum having a high purity starts to crystallize on the surface of the cooling body. The solidificafion proceeds while the eutectic impurities are being released into the liquid phase in the vicinity of the liquid-solid interface to form a diffusion layer. The solidification velocity at this time is governed by the difference between the amount of heat removed from the molten aluminum by the cooling body and the amount of heat supplied to the molten aluminum by heating from outside. Thus the velocity is controlled by these amounts of heat. Further when an increased amount of heat is supplied to the molten aluminum by external heating, with an increased amount of heat removed from the melt by cooling with the cooling body, greater transfer of heat occurs between the cooling body and the melt, consequently giving a greater temperature gradient to the liquid phase in the vicinity of the liquid-solid interface. The greater the temperature gradient, the more effectively is the formation of dendrites inhibited at the interface to prevent the eutectic impurities from being arrested by the dendrites. Ideally, the temperature gradient involved in the liquid phase in the vicinity of the liquid-solid interface should be greater than that of the equilibrium liquidus. The formation of dendrites can then be inhibited completely. From the viewpoint of industrial productivity, however, it is desirable to effect suitable transfer of heat from the molten aluminum to the cooling body by advantageously controlling the external heating and cooling with the cooling body. Further when the cooling body is rotated, the solid phase and the liquid phase move relative to each other, whereby the diffusion layer formed near the liquid-solid interface is effectively agitated and mixed with the other major portion of the liquid phase to disperse the impurities in the diffusion layer throughout the entire liquid phase, consequently greatly reducing the thickness of the diffusion layer. At the same time, the boundary layer in the temperature distribution of the liquid phase is made thinner, consequently permitting the liquid phase to have an increased temperature gradient in the vicinity of the liquid-solid interface. The thicknesses of the diffusion layer and the boundary layer in the temperature distribution can be decreased by increasing the speed of rotation of the cooling body, in other words, the speed of the relative movement between the cooling body and the molten aluminum. However, if the speed is exceedingly high, the aluminum crystallized on the surface of the cooling body is likely to separate off easily due to the increase of the centrifugal force, resulting in reduced productivity. Preferably the speed of the relative movement is within the range of 400 to 8,000 mm/sec because if the speed is lower than 400 mm/sec, the diffusion layer will not be made thinner effectively, whereas if it is higher than 8,000 mm/sec, the increased centrifugal force will lead to reduced productivity. When the cooling body is in the form of a cylinder having a diameter of 160 mm, for example, the body can be rotated at 50 to 1,000 r.p.m., but especially good results are obtained at 200 to 700 r.p.m. Further improved results can be achieved if the direction of rotation of the body is reversed with suitable frequency. Since boron undergoes a eutectic reaction with aluminum, the excess of boron other than the amount of boron forming metallic borides with the peritectic impurities is removed in the same manner as Fe, Si, Cu, Mg and like eutectic impurities.

The high-purity aluminum deposited on the surface of the cooling body on crystallization is recovered, for example, by melting the high-purity fraction or by scraping off the fraction.

According to another aspect of the present invention there is provided a process for producing high purity aluminum comprising the steps of melting the aluminum to be purified and containing both eutectic impurities and peritectic impurities to obtain molten aluminum, and rotating a cooling body when immersed in the molten aluminum while introducing a cooling fluid to the interior of the cooling body to crystallize high-purity aluminum on the surface of the body, characterised by placing the molten aluminum into a boron adding vessel and controlling the temperature of the molten aluminum, adding boron to the molten aluminum within the vessel, continuously agitating the boron-containing molten aluminum, continuously causing the boron-containing molten aluminum to be forwarded to a plurality of purifying tanks from tank to tank and to be discharged from the last tank, and rotating a cooling body at a predetermined speed when immersed in the molten aluminum containing boron and dispersed borides of peritectic impurities resulting from the boron addition within each of the tanks.

This process affords a large quantity of high-purity aluminum efficiently by a continuous operation.

The boron adding vessel and the purifying tanks are prepared, for example, by dividing a single large container into a plurality of sections by partitions each having a communication opening, one of the sections serving as the vessel and the other sections as the tanks. Alternatively a plurality of crucibles may be arranged in a row, with each crucible communicating with another through a trough, such that one of the crucibles serves as the boron adding vessel and the others as the purifying tanks.

Boron is placed into the vessel continuously so that the molten aluminum therein has a constant boron concentration during operation. The molten aluminum in the vessel is agitated to accelerate the reaction between the boron and the peritectic impurities. A cooling body is immersed in the molten aluminum in each of the purifying tanks. The supply of the melt to the purifying tanks is so adjusted that the amount of the melt in each tank remains unchanged during operation. To allow equal amounts of aluminum to crystallize on the surfaces of the cooling bodies in the purifying tanks, the temperature of the molten aluminum, the speed of rotation and cooling capacity of the cooling bodies are suitably controlled. The eutectic impurity concentration of the molten aluminum in the purifying tanks progressively increases from tank to tank away from the melting furnace. The average impurity concentration of all the aluminum fractions obtained is variable by varying the ratio of the total amount of aluminum fractions recovered by the cooling bodies to the total amount of the melt supplied. (The ratio will be referred to as "recovery ratio"). The smaller the recovery ratio, the lower is the average impurity concentration. Accordingly aluminum having a constant purity which is higher than the purity of the original aluminum supplied from the melting furnace for purification can be obtained by rendering the recovery ratio constant. Further at the same recovery ratio, the purity of the aluminum obtained increases with the increase in the number of purifying tanks.

Embodiments of the present invention will now be described by way of example only with reference to the accompanying drawings, in which:-
Fig. 1 is a view in vertical section showing a first embodiment of apparatus for producing high-purity aluminum by the process of the invention;
Fig. 2 is a view in vertical section showing a second embodiment of apparatus for producing high-purity aluminum by the process of the invention;
Fig. 3 is an enlarged fragmentary view of Fig. 2 partly broken away;
Fig. 4 is a graph showing the result achieved when the process of the invention was practiced with use of the second apparatus, the graph showing the relation of the amount of aluminum (yield) crystallized on the peripheral surface of a cooling body in each purifying tank to the ratio of the eutectic impurity concentration of the molten aluminum in the tank to the eutectic impurity concentration of the aluminum to be purified; and
Fig. 5 is a graph showing the relation between the number of purifying tanks and the ratio of the eutectic impurity concentration of the aluminum obtained to that of the aluminum to be purified, the relation being determined by practicing the process of the invention with use of the second apparatus.

With reference to a first apparatus for practicing the process of the invention, the aluminum to be purified and containing both eutectic impurities and peritectic impurities is melted and placed in a molding container comprising a crucible 2. The molten aluminum 1 is heated and maintained at a temperature exceeding the solidifying temperature thereof. Boron is added to the molten aluminum 1, and the mixture is agitated for at least 5 minutes. A cooling body 3 is thereafter immersed in the melt 1. The cooling body 3 is in the form of a hollow cylinder having closed opposite ends and is movable upward and downward. A hollow rotary shaft 4 extends upward from the upper end of the body 3. The interior of the hollow rotary shaft 4 is in communication with the interior of the cooling body 3. A cooling fluid supply pipe 5 extends through the shaft 4 into the cooling body 3. The rotary shaft 4 is provided at its upper end with a drive device (not shown), by which the shaft 4 and the body 3 are rotated. The top and bottom of the body 3 and the portion of the shaft 4 to be exposed to the melt 1 are preferably covered with a heat insulating material 6 so as not to permit aluminum to crystallize on these portions. This is due to the reason that since the effect produced by the rotation of the body 3 is lower at these portions than at the periphery of the body 3, aluminum, if crystallizing on these portions will have a lower purity than the aluminum crystallizing on the periphery. The cooling body 3 is rotated while introducing a cooling fluid, such as air, nitrogen or argon, from the pipe 5 into the body 3 at an adjusted rate so that the portion of the melt 1 around the body 3 will be cooled slowly. Pro-eutectic aluminum having a high purity then starts to crystallize on the periphery of the body 3. After a specified quantity of aluminum has been deposited on the body 3, the body is raised and withdrawn from the melt 1, and the high-purity aluminum obtained is collected.

The above procedure is repeated in aluminum melts of progressively higher purities to obtain aluminum of greatly improved purity.

With reference to Figs. 2 and 3 showing a second apparatus, there is provided a melting furnace 11 for melting the aluminum to be purified and containing both eutectic impurities and peritectic impurities. A large container 12 in the form of a horizontally elongated rectangular parallelepiped is disposed on the right side of the furnace 11. The container 12 is divided into five sections by partitions 13. Of these sections, the one at the left end serves as a boron adding vessel 14, and the other four sections serve as purifying tanks 15 to 18. The partitions 13 are formed at their upper ends with openings 19 through which the vessel 14 and the tanks 15 to 18 communicate with one another. The vessel 14 has an agitator 20 in its interior. The agitator 20 comprises a vertical rotary shaft 21, a propeller- shaped stirring blade 22 attached to the lower end of the shaft 21 and unillustrated drive means. Each of the tanks 15 to 18 is provided with a cooling body 23 which is movable upward and downward. The body 23 is in the form of a downwardly tapered hollow cylinder having closed opposite ends and a hollow rotary shaft 24 extending upward from its top. The interior of the shaft 24 is in communication with the interior of the body 23. A cooling fluid supply pipe 26 extending through the shaft 24 into the body 23 has a large number of cooling fluid outlets 25 in its peripheral wall. The upper end peripheral portion and the bottom of the cooling body 23 are covered with heat insulating members 27 and 28 respectively.

Before molten aluminum 30 is placed into the tanks 14 to 18, the cooling bodies 23 are held raised as indicated in broken lines in Fig. 2.

The aluminum to be purified and containing both eutectic impurities and peritectic impurities is melted in the furnace 11, and the molten aluminum 30 is first placed into the vessel 14, in which boron is added to the melt 30. The mixture is agitated by the agitator 20. In this vessel 14, the boron reacts with Ti, V, Zr and like peritectic impurities, forming TiB₂, VB₂, ZrB₂ and like insoluble metallic borides. The molten aluminum containing the eutectic impurities, insoluble metallic borides and an excess of boron flows into the tanks 15 to 18 through the communication openings 19. After a predetermined amount of molten aluminum 30 has been placed into each of the tanks 15 to 18, the cooling body 23 is lowered and immersed in the melt, with the upper heat insulating member 27 in contact with the melt 30 and with the lower edge of the member 27 located within the mass of the melt 30 at such a position that it will not be influenced by the temperature of the atmosphere. The upper end peripheral portion of the body 23 is covered with the insulating member 27, and the body is so immersed in the melt 30 that the member 27 is in contact with the surface of the melt 30 with its lower edge at a position where it is free of the influence of the atmospheric temperature, for the following reason. The portion of the melt 30 near the surface thereof exposed to the atmosphere has a lower temperature than the other portion by being affected by the atmospheric temperature and is therefore liable to solidify on the periphery of the body 23 in the vicinity of the above surface. Consequently aluminum solidifies at a higher velocity at this portion than at the other portion of the periphery of the body 23, with the result that the aluminum fraction deposited on this portion has a lower purity than the fraction on the other portion and becomes mixed with the latter fraction when the purified aluminum is removed from the outer periphery of the body 23 for collection after the completion of the purifying operation. This results in a reduced overall purifying efficiency. Further the bottom of the cooling body 23 is covered with the heat insulating member 28 because the rotation of the body 23 will not produce a satisfactory effect at the bottom, such that the aluminum fraction deposited on the bottom of the body 23 has a lower purity than the other fraction on the periphery of the body.

The cooling body 23 in this state is rotated while injecting a cooling fluid into the body through the inlets 25 of the supply pipe 26. This causes aluminum to crystallize on the portion of the peripheral surface of the body 23 which is immersed in the melt 30 and which is not covered with the insulating members 27 and 28. Since the metallic borides contained in the melt 30 are centrifugally forced away from the body 23 by the rotation thereof, the aluminum deposited on the periphery of the body 23 is free from such borides. The excess of boron, which forms a eutectic with aluminum, is removed like the eutectic impurities. The temperature of the molten aluminum, and the speed of rotation and cooling capacity of the bodies 23 are so controlled that equal amounts of aluminum will be deposited on the peripheral surfaces of the bodies in the purifying tanks 15 to 18, while the supply and discharge of molten aluminum are controlled so that the tanks 15 to 18 contain equal amounts of melt with the recovery ratio maintained at a constant value. Assuming that the molten aluminum supplied from the furnace 11 has a eutectic impurity concentration of CO and that the melt portions contained in the tanks 15 to 18 have eutectic impurity concentrationa of C1, C2, C3 and C4 respectively, Further the ratio of the eutectic impurity concentration of the melt in each of the tanks 15 to 18 to C0, namely the ratio CN/CO where N is 1 to 4, increases with the start of the operation but levels off when the amount of aluminum deposit on the periphery of the cooling body 23 reaches a value as shown in Fig. 4. At this time, the total amount of eutectic impurities, Ms, in the aluminum recovered by the cooling bodies 23 plus the amount of eutectic impurities, Mn, in the molten aluminum discharged from the tank 18 at the right end is always equal to the amount of eutectic impurities, Mo, in the aluminum to be purified. Accordingly, if the eutectic impurity concentration and the effective distribution coefficient of the eutectic impurities of the molten aluminum in each of the tanks 15 to 18 are known, high-purity aluminum can be obtained with the desired eutectic impurity concentration when the recovery ratio is set to a definite value. The smaller the recovery ratio, the lower is the eutectic impurity concentration of the molten aluminum in each purifying tank, so that the cast block obtained has a higher purity. The purity of the aluminum to be obtained can be determined by varying the recovery ratio. At a definite recovery ratio, the eutectic impurity concentration of the molten aluminum discharged increases with the increase of the number of purifying tanks as seen in Fig. 5, enabling the cooling bodies 23 to afford aluminum of higher purity.

When the same operation as above is repeated again with use of the aluminum collected by the cooling bodies 23, aluminum having a higher purity can be obtained. Since the molten aluminum resulting from the second operation usually has a higher purity than the original aluminum used as the material for the first operation, the molten aluminum, if returned to the furnace 11, gives an improved yield.

### Example 1

The apparatus shown in Fig. 1 was used. Aluminum containing 0.08 wt.% of Fe, 0.05 wt.% of Si, 0.0015 wt.% of Ti, 0.004 wt.% of V and 0.0005 wt.% of Zr was melted, and the molten aluminum 1 was maintained at 670°C in the crucible 2. AI-3 wt.% B master alloy was added to the alumimum 1 so that the resulting melt had a boron concentration of 0.004 wt.%. The mixture was agitated for 5 minutes after the addition of the alloy. The cooling body 3, 100 m in outside diameter, was immersed in the melt 1 and rotated at a speed of 400 r.p.m. while supplying air into the body 3 through the supply pipe 5. The body 3 was rotated for 10 minutes and thereafter withdrawn from the melt 1 by raising. The body 3 was found to have aluminum deposited on its periphery in an amount of 20 wt.% based on the amount of the original aluminum. When checked for impurity concentration, the cast aluminum block was found to contain 0.008 wt.% of Fe, 0.012 wt.% of Si, less than 0.0001 wt.% of Ti, 0.0002 wt.% of V, less than 0.0002 wt.% of Zr and 0.0003 wt.% of B.

### Example 2

The apparatus shown in Fig. 1 was also used. Aluminum containing 0.08 wt.% of Fe, 0.05 wt.% of Si, 0.002 wt.% of Ti, 0.008 wt.% of V and 0.001 wt.% of Zr was melted, and the molten aluminum 1 was maintained at 670°C in the crucible 2. AI-3 wt.% B master alloy was added to the aluminum 1 so that the resulting melt had a boron concentration of 0.008 wt.%. The mixture was agitated for 5 minutes after the addition of the alloy. The cooling body 3, 200 mm in outside diameter, was then immersed in the melt 1 and rotated at a speed of 650 r.p.m. while supplying air into the body through the pipe 5. After rotating the body 3 for 10 minutes, the body 3 was withdrawn from the melt. The body 3 was found to have aluminum deposited on its periphery in an amount of 20% based on the amount of the original aluminum. When checked for impurity concentration, the cast aluminum block was found to contain 0.005 wt.% of Fe, 0.009 wt.% of Si, less than 0.0001 wt.% of Ti and V, less than 0.0002 wt.% of Zr and 0.0005 wt.% of B.

### Example 3

The apparatus shown in Figs. 2 and 3 was used. The cooling bodies 23 were held raised. Aluminum containing 0.08 wt.% of Fe, 0.05 wt.% of Si. 0.002 wt.% of Ti and 0.008 wt.% of V was melted in the furnace 11, and the molten aluminum was supplied to the boron adding vessel 14. Boron was added to the aluminum so that the resulting melt had a boron concentration of 0.008 wt.% at all times. The mixture was agitated by the agitator 20. When the purifying tanks 15 to 18 were filled with the molten aluminum flowing through the communication openings 19, each cooling body 23 having a diameter of 200 mm at the portion thereof covered with the heat insulating member 27 was lowered into the molten aluminum 30. The body 30 was rotated at 400 r.p.m. while supplying a cooling fluid into its interior from the pipe 26. During operation, the molten aluminum was continuously supplied from the furnace 11 to the vessel 14 and tanks 15 to 18 so as to fill up these containers to a constant level. Boron was also continuously placed into the vessel 14 to maintain the boron concentration at 0.008 wt.% at all times. The eutectic impurity concentrations C1, C2, C3 and C4 of the melt portions in the tanks 15 to 18 remained in the relation of C1, C2, C3, C4 from the start of the operation, and a steady state was established after the amount of aluminum deposit on the body 23 reached a specified amount. When the effective distribution coefficient of iron was 0.1 at a recovery ratio of 0.7, the ratios of the iron concentrations C1, C2, C3 and C4 to the iron concentration CO of the molten aluminum supplied from the furnace 11, namely C1/CO, C2/CO, C3/CO and C4/C0, levelled off at 1.3, 1.6, 2 and 2.7, respectively. The operation was continued in this state. When checked for impurity concentration, the resulting cast aluminum blocks were found to contain 0.008 wt.% of Fe, 0.008 wt.% of Si, 0.0001 wt.% of Ti, 0.0002 wt.% of V and 0.0006 wt.% of B on the average.

### Example 4

The operation of Example 3 was repeated under the same conditions except that the recovery ratio was 0.4. The operation was continued in a steady state. All the aluminum blocks obtained were found to have average impurity concentrations of: 0.005 wt.% Fe, 0.006 wt.% Si, 0.0001 wt.% Ti, 0.0002 wt.% V and 0.0005 wt.% B.

### Example 5

The operation of Example 3 was repeated under the same conditions as in Example 3 except that eight purifying tanks were used in place of the four tanks. The operation was continued in a steady state. The aluminum blocks obtained were found to have the following average impurity concentrations: 0.0065 wt.% Fe, 0.007 wt.% Si, 0.0001 wt.% Ti, 0.0002 wt.% V, 0.0005 wt.% B. The aluminum had a higher purity than that obtained in Example 3 with use of the four purifying tanks and was produced at twice the speed therein.

## Claims

1. A process for producing high-purity aluminum comprising the steps of melting the aluminum to be purified and containing both eutectic impurities and peritectic impurities to obtain molten aluminum, and rotating a cooling body when immersed in the molten aluminum while introducing a cooling fluid to the interior of the cooling body to crystallize high-purity aluminum on the surface of the body, characterised by placing the molten aluminum into a holding container (2) and controlling the temperature of the molten aluminum, adding boron to the molten aluminum within the container (2), and rotating the cooling body (3) at a predetermined speed when immersed in the molten aluminum containing boron and dispersed borides of peritectic impurities resulting from the boron addition.

2. A process according to claim 1, characterised in that the speed of the relative movement between the cooling body (3) and the molten aluminum is about 400 to about 8,000 mm/sec when the cooling body is rotated.

3. A process for producing high purity aluminum comprising the steps of melting the aluminum to be purified and containing both eutectic impurities and peritectic impurities to obtain molten aluminum, and rotating a cooling body when immersed in the molten aluminum while introducing a cooling fluid to the interior of the cooling body to crystallize high-purity aluminum on the surface of the body, characterised by placing the molten aluminum into a boron adding vessel (14) and controlling the temperature of the molten aluminum, adding boron to the molten aluminum within the vessel

(14), continuously agitating the boron-containing molten aluminum, continuously causing the boron-containing molten aluminum to be forwarded to a plurality of purifying tanks (15-18) from tank to tank and to be discharged from the last tank (18), and rotating a cooling body (23) at a predetermined speed when immersed in the molten aluminum containing boron and dispersed borides of peritectic impurities resulting from the boron addition within each of the tanks (15-18).

4. A process according to claim 3, characterised in that the supply and the discharge of the molten aluminum are controlled so that the amounts of the molten aluminum in the purifying tanks (15-18) remain unchanged during operation, and the cooling bodies (23) are controlled so that equal amounts of high-purity aluminum are crystallized on the surfaces of the cooling bodies (23).

5. A process according to any of claims 3 or 4, characterised in that the speed of the relative movement between the cooling body (23) and the molten aluminum is about 400 to about 8,000 mm/sec when the cooling body is rotated.

## Patentansprüche

1. Verfahren zum Herstellen von hochreinem Aluminium, bei dem das zu reinigende und sowohl eutektische Verunreinigungen als auch peritektische Verunreinigungen enthaltende Aluminium zum Erhalt von geschmolzenem Aluminium geschmolzen wird und bei dem ein in das geschmolzene Aluminium eingetauchter Kühlkörper rotiert wird, während man ein Kühlfluid in das Innere das Kühlkörpers einführt, damit sich hochreines Aluminium an der Oberfläche des Körpers kristallisiert, dadurch gekennzeichnet, daß man das geschmolzene Aluminium in einen Haltebehälter (2) einbringt und die Temperatur des geschmolzenen Aluminiums steuert, Bor zu dem geschmolzenen Aluminium innerhalb des Behälters (2) hinzufügt und den Kühlkörper (3) mit einer vorbestimmten Geschwindigkeit rotiert, wenn er in das aufgrund der Borzugabe Bor und dispergierte Boride von peritektischen Verunreinigungen enthaltende geschmolzene Aluminium eingetaucht ist.

2. Verfahren nach Anspruch 1, dadurch gekennzeichnet, daß die Geschwindigkeit der Relativbewegung zwischen dem Kühlkörpers (3) und dem geschmolzenen Aluminium etwa 400 bis etwa 8000 mm/sec beträgt, wenn der Kühlkörpert rotiert wird.

3. Verfahren zum Herstellen von hochreinem Aluminium, bei dem das zu reinigende und sowohl eutektische Verunreinigungen als auch peritektische Verunreinigungen enthaltende Aluminium zum Erhalt von geschmolzenem Aluminium geschmolzen wird und bei dem ein in das geschmolzene Aluminium eingetauchter Kühlkörper rotiert wird, während man ein Kühlfluid in das Innere des Kühlkörpers einführt, damit sich hochreines Aluminium an der Oberfläche des Körpers kristallisiert, dadurch gekennzeichnet, daß man das geschmolzene Aluminium in ein Borzugabegefäß (14) einbringt und die Temperatur des geschmolzenen Aluminiums steuert, Bor zu dem geschmolzenen Aluminium innerhalb des Gefäßes (14) hinzufügt, das Bor enthaltende geschmolzene Aluminium kontinuierlich in Bewegung hält, das Bor enthaltende geschmolzene Aluminium kontinuierlich zu einer Mehrzahl von Reinigungstanks (15 bis 18) von Tank zu Tank vorfördert und aus dem letzten Tank

(18) entnimmt und innerhalb jedes Tanks (15 bis 18) einen Kühlkörper (23) mit einer vorbestimmten Geschwindigkeit rotiert, wenn er in das aufgrund der Borzugabe Bor und dispergierte Boride von peritektischen Verunreinigungen enthaltende geschmolzene Aluminium eingetaucht ist.

4. Verfahren nach Anspruch 3, dadurch gekennzeichnet, daß das Zuführen und das Abführen des geschmolzenen Aluminiums in der Art gesteuert werden, daß die Mengen geschmolzenen Aluminiums in den Reinigungstanks (15 bis 18) während des Betriebs unverändert bleiben, und daß die Kühlkörper (23) derart gesteuert werden, daß an den Oberflächen der Kühlkörper (23) gleiche Mengen von hochreinem Aluminium kristallisiert werden.

5. Verfahren nach einem der Ansprüche 3 oder 4, dadurch gekennzeichnet, daß die Geschwindigkeit der Relativbewegung zwischen dem Kühlkörper (23) und dem geschmolzenem Aluminium etwa 400 bis etwa 8000 mm/sec beträgt, wenn der Kühlkörper rotiert wird.

## Revendications

1. Procédé d'obtention d'aluminium à haute pureté, consistant à fondre l'aluminium à purifier et contenant des impuretés eutectiques et des impuretés péritectiques, pour obtenir de l'aluminium fondu, à faire tourner un élément de refroidissement immergé à l'intérieur de l'aluminium fondu, avec introduction d'un fluide réfrigérant à l'intérieur de l'élément de refroidissement, afin de réaliser la cristallisation d'aluminium à haute pureté sur la surface de l'élément, caractérisé en ce qu'il consiste à placer l'aluminium fondu à l'intérieur d'un récipient (2), à contrôler la température de l'aluminium fondu, à ajouter du bore à l'aluminium fondu à l'intérieur du récipient (2), à faire tourner l'élément de refroidissement à une vitesse prédéterminée, lorsqu'il est immergé dans l'aluminium fondu, contenant le bore et des borures dispersés d'impuretés péritectiques résultant de l'addition de bore.

2. Procédé selon la revendication 1, caractérisé en ce que la vitesse du mouvement relatif entre le corps de refroidissement (3) et l'aluminium fondu est de l'ordre de 400 à 8,000 mm/sec lorsque l'élément de refroidissement est animé d'un mouvement de rotation.

3. Procédé d'obtention d'aluminium à haute pureté, comprenant les phases consistant à fondre l'aluminium à purifier et contenant, à la fois, des impuretés eutectiques et des impuretés péritectiques pour obtenir de l'aluminium fondu, à faire tourner un élément de refroidissement, lorsqu'il est immergé dans l'aluminium fondu avec introduction d'un fluide réfrigérant à l'intérieur du corps de refroidissement pour réaliser la cristallisation d'un aluminium à haute pureté sur la surface de l'élément, caractérisé en ce qu'il consiste à placer l'aluminium fondu dans un récipient (14) destiné à l'addition du bore, à contrôler la température de l'aluminium fondu, à ajouter le bore à l'aluminium fondu à l'intérieur de ce récipient (14), à agiter en continu l'aluminium fondu contenant le bore, à transférer en continu l'aluminium contenant le bore vers une pluralité de réservoirs de purification (15-18) de réservoir en réservoir, avec évacuation hors du dernier réservoir (18), et à faire tourner l'élément de refroidissement (23) à une vitesse prédéterminée lorsqu'il est immergé dans l'aluminium fondu contenant le bore et les borures d'impuretés péritectiques, résultant de l'addition de bore, dispersés dans chaque réservoir (15-18).

4. Procédé selon la revendication 3, caractérisé en ce qu'il consiste à contrôler d'alimentation et l'évacuation d'aluminium fondu, de telle sorte que les quantités d'aluminium fondu dans les divers réservoirs de purification (15-18) demeurent inchangées au cours de l'opération, et en ce que les éléments de refroidissement (23) sont contrôlés de telle sorte que des quantités égales d'aluminium à haute pureté sont cristallisées sur les surfaces de leurs corps respectifs.

5. Procédé selon l'une des revendications 3 ou 4, caractérisé en ce que la vitesse du mouvement relatif entre l'élément de refroidissement (23) et l'aluminium fondu est de l'ordre de 400 à 8,000 mm/sec lorsque l'élément de refroidissement est entraîné en rotation.
